

No. 836,587.

PATENTED NOV. 20, 1906.

D. LANCE.

## WET METHOD OF EXTRACTING COPPER, ZINC, &c., FROM THEIR ORES.

APPLICATION FILED AUG. 7, 1905.

2 SHEETS—SHEET 1.

High.



*Witnesses:*

L. Waldman  
C. H. Crawford

Inventor  
Denis Lance  
by B. Singer Attorney.

No. 836,587.

PATENTED NOV. 20, 1906.

D. LANCE.

## WET METHOD OF EXTRACTING COPPER, ZINC, &c., FROM THEIR ORES.

APPLICATION FILED AUG. 7, 1905.

2 SHEETS—SHEET 2.



## *Witnesses.*

L. Waldman  
C. H. Crawford

Inventor.  
Denis Lance  
by P. Singer Attorney.

# UNITED STATES PATENT OFFICE.

DENIS LANCE, OF PARIS, FRANCE.

## WET METHOD OF EXTRACTING COPPER, ZINC, &c., FROM THEIR ORES.

No. 836,587.

Specification of Letters Patent.

Patented Nov. 20, 1906.

Application filed August 7, 1905. Serial No. 273,063.

*To all whom it may concern:*

Bé it known that I, DENIS LANCE, a citizen of the French Republic, and a resident of Paris, France, have invented certain new and useful improvements in methods of extracting copper, zinc, cadmium, silver, nickel, cobalt, and tungsten in the form of hydrated oxids direct from their ores by wet process, of which the following is a specification.

10 Simple or complex silicates may be rendered manageable by ammoniacal solutions, aminic solutions or ammoniaco-aminic solutions, if they be previously decomposed by a powerful acid acting alone or assisted by heat.

15 In treating nickel ores containing silicic acid, and particularly those from New Caledonia, Silesia, and Russia it is advisable for the purpose of quickly affecting the ore and 20 at the same time rendering the effect more complete, to add to the ore, a certain quantity of a chlorid which is easily decomposed by sulfuric acid, and for this purpose to employ in place of pure acid strongly-nitrous acid in the state in which it leaves the Gay-Lussac tower.

25 In consequence of the reaction of the nitrous sulfuric acid on the chlorids, nitrosyl chlorid  $\text{NOCl}$ , as likewise nitryl chlorid  $\text{NO}_2\text{Cl}$  is generated, and these chloro-nitrates act rapidly on the ore containing silicic acid, and, in combination with the metals contained in this ore, form chlorids, setting free nitrogen dioxid (or nitric oxid)  $\text{NO}$  and the 30 peroxid of nitrogen  $\text{NO}_2$  contained in the nitrosyl chlorid and in the nitryl chlorid. Again, these metallic chlorids, being immediately decomposed by the nitrous sulfuric acid, the compounds  $\text{NOCl}$  and  $\text{NO}_2\text{Cl}$  are 35 continually regenerated and the action on the ore proceeds perfectly.

40 The operation being carried on in a closed vessel, it will be understood that very small quantities of chlorids and of nitrous products are sufficient for affecting very considerable quantities of ore. Moreover, the compounds  $\text{NOCl}$  and  $\text{NO}_2\text{Cl}$  being rather volatile and almost insoluble in water at the temperature of the reaction, they can be 45 easily collected when the apparatus is emptied. It has likewise been observed that the salts which are formed during these reactions contain from six to seven molecules of water. The acid which is employed is quickly dehydrated, and the salts which are formed not 50 being very soluble in water a protective

coating is formed around each portion of ore and quickly restricts the action. It is accordingly necessary during this action to introduce quantities of water proportional thereto, so that the density of the acid is kept between  $40^{\circ}$  and  $50^{\circ}$  Baumé if a good yield be desired. This action is further promoted if during its progress the pulverizing of the ore be continued, as if this be done any protective layer of salts which may form around portions of the ore is destroyed by the pulverizing operation. Moreover, it has been observed that the yield, other things being equal, is greatest if the acid employed be previously heated to a temperature of  $110^{\circ}$  to  $120^{\circ}$ . Finally, it should be mentioned that it is desirable in the last stages of the reaction to employ a solution of a bisulfate instead of simple water for the purposes of hydration.

55 The observations referred to have led to a particular process which will be described, as employed, for example, in the treatment of a New Caledonian nickel ore containing 60 silicic acid.

65 In the accompanying diagram the whole of the operations can be followed; Figure 1 representing the first part of the installation and Fig. 2 the second part. These two parts can 70 be joined together at the places indicated by broken lines in the two figures.

75 1 is a pyrite or soda furnace fed by means of the feed device 2 and provided at 3 with retorts for the manufacture of the nitric acid. 80 These retorts are heated by the waste heat and supplied with nitrate by the feed device 4. The nitric-acid vapors and the sulfurous-acid vapors, as well as the necessary oxygen for the manufacture of the sulfuric acid, enter 85 the first lead-chamber 6 through the pipe 5. They there mix with the steam coming from the boiler 7 through the pipe 8. The chambers 9 and 10 are two ordinary lead-chambers, where the reactions take place.

90 100 11 is a Gay de Lussac tower. The acid manufactured in the chambers 10, 9, and 6 reaches the top of the Gay de Lussac tower through the pipe 12. The nitrous sulfuric acid passes out at the bottom of the tower through the pipe 13, while the nitrogen and the oxygen in excess escape through the pipe 14 into the chimney. The nitrous sulfuric acid passes through the pipe 13, not into a Glover 105 tower, but into the apparatus for sulfating the ore, which takes the place thereof. These apparatuses consist of Alsing cylinders 16

and 17, each having a leaden casing, a porcelain lining, and containing lumps of silex and furnished with axial pipes. To these cylinders the feed device 19 conveys the ore, which 5 has been previously crushed, while the feed device 21 conveys to the cylinders the chloridated solution coming from the tank 20, and which may be sea-water, for example, sufficiently concentrated. This "chloridated" solution flows through the pipe 21'. As the action proceeds water is added by means of pipes 22, running from the main pipe 23, the bisulfate—for example, the bisulfate of soda proceeding from the manufacture of the nitric acid—being added by means of the feed devices 24 and 19.

For the purpose of heating the collection of apparatus and the acid to the temperature most favorable for the reaction, hot air, coming from the flue 27 of the boiler 7, is caused to circulate in the Alsing cylinders 16 17 by means of the pump 25 and the pipe 26. This air passes out through the pipe 28 and comes under the fire-bars of the sulfurous-acid furnace, so that if in its passage it has taken up any nitrous vapors these vapors are restored to what is circulating generally in the lead-chambers.

When the operation of sulfating the ore is 30 finished—that is, after the action has continued from one-half to five hours, according to the nature of the ores—the nitrated compounds and chloro-nitrated compounds are discharged through the pipe 29 into the pipe 5, from which they pass into the lead-chambers 6 9 10. The nitryl chlorid and nitrosyl chlorid play the same part (in fact, a more active part) in the manufacture of sulfuric acid as is played by the nitrosyl sulfate with 40 which this manufacture is usually effected.

The Alsing cylinders, in which the sulfating operation is effected, thus act in the same way as the Glover tower, which, moreover, they replace, the nitrous or chloro-nitrous 45 products being recovered in the cylinders at the end of the reaction and restored to the lead-chamber and the sulfuric acid being discharged in the form of sulfate of the dissolved metals.

50 With the exception of the losses in working inherent in the manufacture of sulfuric acid the nitrous and chloro-nitrous products are constantly regenerated.

Instead of hot air coming from the flue 27 being caused to circulate in the Alsing cylinders the mixture of sulfurous acid, nitric acid, and air which enters the first lead-chamber 6 may be introduced direct into these apparatuses. These gases, the Glover tower 55 being dispensed with, are, in fact, at a high temperature, too great for allowing of their being utilized in the lead-chambers without previous cooling, which would render it necessary to make the pipe 5, leading from the furnace 1 to the lead-chamber 6, rather long. By

conveying these gases into the Alsing cylinders the greater part of this waste heat is utilized. On the other hand, they will issue charged with nitrous and chloro-nitrous vapors which were previously conveyed through 70 the pipe 29 into the conduit 5 in order to mix with them. Moreover, as they take up steam coming from the acid in the Alsing cylinders it is necessary, as when a Glover tower is employed, to provide the lead-chamber with a 75 smaller quantity thereof. Under these conditions the collection of Alsing cylinders, in which the ore is treated most exactly and completely, replaces the Glover tower, the pulverised ore and the lumps of silex replacing the brick filling and the acid passing out freed from nitrous and chloro-nitrous products in the form of sulfate of the metals which had to be dissolved. Thus the economical advantages of that tower are utilized 80 alike in the sulfating of the ore and in the manufacture of nitrous and chloro-nitrous sulfuric acid. The nitrous or chloro-nitrous gases having been carried off, the Alsing cylinders 16 and 17 are tilted in the hollow 85 90 and the contents thereof flow through the gutter 31 into the stirring-tank 32, which is constructed in masonry and covered with lead. The sulfated mass passes through the pump 33 and, through the medium of the 95 pipe 34, flows alternately into one or the other of the filter-presses 35. The nickeliferous solution flows into the receptacles 36, then through the pipe 37 into the stirring-tank 38. The "cake" residue is emptied into the stirring-tank 39, situated below the filter-presses 35 and after having been diluted with water entering through 40, and resulting from the last washing, passes through the filter-presses 41, through the pump 42, and the pipe 43. 100 The second nickeliferous solution thus obtained is likewise conveyed to the tank 38 by means of vessels 44 and pipes 45 and 37. The cake, as previously, is emptied into the tank 46 and steeped in the ordinary water 105 coming through 47. The diluted mass is taken up by the pump 48 and passes to the press-filters 50 through the pipe 49. The small quantities of nickeliferous solution coming from the filter-presses 50 are conveyed, as 110 was previously seen, to the last tank 39 by means of the vessels 51 and the pipe 40. The exhausted sterile mass is thrown into the gutter 52 and discharged through the central drain 53. The nickeliferous solution concentrated 115 in 38 has an addition made to it at first of carbonate of lime (ordinary limestone pulverized dry or moist) contained in the hopper 54, fed by the device 55, so as to effect the saturation of the greater part of the dissolved salts. This 120 saturation is completed by the addition of thin milk of lime coming from the tank 56, fed by the device 57. During this operation a vigorous agitation is maintained in the tank 38. The precipitation having been finished, 130

the mass is conveyed to the filter-presses 58 through the medium of the pump 59 and the pipe 60. The liquid coming from the filter-presses 58, and which should not cause any reaction in the soluble sulfids, is discharged 5 through the vessels 61 and the pipe 62 into the central drain 53. The nickeliferous calcic precipitate is emptied into the hopper 63 of the feed device 64 and conveyed above the lixiviating-cylinders 65 66 67, resembling chloridating-casks. These cylinders 65 66 67 being charged, an ammoniacal solution of 22° Baumé, coming from the tank 68, is introduced into them by means of the pump 69 15 and the pipe 70. This solution may be introduced into all the apparatuses at once; but it is better to charge from one to the other and produce a methodical circulation of the fluid, so that the liquor having remained a certain 20 time in 65 passes into 66, then into 67, and into the following apparatus if there be such, and passes out completely saturated with oxid of nickel. In this way the cake is completely exhausted with the minimum of ammonia, and it is then sufficient if distillation 25 be effected on the minimum of liquid.

The lixiviation having been effected in one apparatus, this being ascertained by taking samples, the ammonia containing the sterile calcic matter is recovered by heating the 30 mass at 100°, which can be effected by means of the steam-pipe 71, after, however, the largest possible quantity of liquid has been expelled through the filtering-section 72 by means of the compressed air entering through 35 73. This expulsion may also be effected by the steam. The ammonia-gas coming from the lixiviating apparatus during this operation passes through the pipe 74 to the pipe 40 75, which collects the gases from the distilling-column 76. The nickeliferous ammoniacal solutions reach this same column through the pipe 77; but instead of reaching it direct they pass into the closed temperature-changers 78 79 through the pipe 80 and finally 45 reach the top of the column through the pipe 81. They are thus gradually heated. The column is heated by a steam-jet coming through the pipe 82, which branches off 71. The ammonia-gas coming from the column, 50 as well as that passing through 74 from the lixiviating-cylinders or any other part, passes through the pipe 75 to the temperature-changer 79. It circulates in the coil-pipe 83, 55 then flows through the pipe 84 to the bottom of the condenser. Into this condenser, at the top, ordinary water enters through 86 or residuary water resulting from a previous operation and entering through 87. The regenerated ammoniacal solution flows through 88 into the tank 68. The cycle is thus completed. The precipitated oxid of nickel 60 passes out with the residuary hot water from the column 76 through the pipe 89 and by means of the pump 90 and the pipe 91 this 65

collection is conveyed to the filter-presses 92, which are provided with hermetically-closed casings. The oxid of nickel remains between the plates, (or stages,) and the residuary water discharged into the casing passes through the 70 pipe 93 into the coil-pipe 94 from the temperature-changer 78 and flows in a cold state through the pipe 87 at the top of the condenser, so that if in consequence of imperfect distillation or bad filtration they retain any 75 oxid of nickel or ammonia, or both at once, these products reenter the general circulation without any loss being possible. The oxid of nickel is washed, if necessary, with ordinary water flowing from 86 or with the steam 80 coming from 71, then emptied into the hopper 94 of a feed device 95, which conveys it to ordinary reducing apparatus.

If the washing be effected with water, the washing-waters issuing from 93 are combined 85 with the residuary waters. If the washing be effected by steam, the small quantities of ammonia-gas pass through the pipe 96 and the pipe 74 and rejoin the gases issuing from the column 76. The losses of ammonia, as of 90 nickel, may thus be considered as reduced to the smallest quantity possible in working. This collection of reactions and of apparatus is employed in the same manner as when complex, sulfurous, antimonious, or arsenic anti-monious ores are treated instead of ores containing silicic acid. 95

Having now fully described my said invention, what I claim, and desire to secure by Letters Patent, is—

100

1. The herein-described process of extracting and concentrating metals from ores consisting in decomposing ores with conjointly-reacting nitro-sulfuric acid, decomposable metallic chlorids, nitro-chlorids, oxids of nitrogen fumes, oxid of sulfur fumes and water vapors, in effecting hydration of the herefrom-resulting salts of the metals contained in said ores, in separating said hydrated material and saturating with calcareous reagents, in separating the metalliferous calcareous precipitate and lixiviating with ammonia solutions, in removing the calcareous precipitate, in distilling the lixiviation fluid, and in separating the precipitated metallic oxids. 110

115

2. The herein-described process of extracting and concentrating metals from ores consisting in treating ores with nitrosulfuric acid and decomposable metallic chlorids, in causing nitrosulfuric acid to react upon decomposable metallic chlorids to form nitrochlorids, in causing the said nitrochlorids to react upon the metal contained in said ore to form the chlorid of such metal, in causing the previously-added nitrosulfuric acid to react 120 upon the said metal chlorid to form the sulfate of the metal contained in said ore.

120

3. The herein-described process of extracting and concentrating metals from ores consisting in treating ores with nitrosulfuric acid 130

and decomposable metallic chlorids in closed reaction-chambers, in causing nitrosulfuric acid to react upon decomposable metallic chlorids to form nitrochlorids, in causing the said nitrochlorids to react upon the metal contained in said ore to form the chlorid of such metal, in causing the previously-added nitrosulfuric acid to react upon the said metal chlorid to form the sulfate of the metal contained in said ore, in heating to 110° to 120° centigrade to effect distillation of the aforementioned nitrochlorids and in injecting oxid-of-sulfur fumes and water-vapors to form new quantities of sulfuric acid.

4. The herein-described process of extracting and concentrating metals from ores consisting in treating ores with nitrosulfuric acid and decomposable metallic chlorids in closed reaction-chambers, in causing nitrosulfuric acid to react upon decomposable metallic chlorids to form nitrochlorids, in causing the said nitrochlorids to react upon the metal contained in said ore to form the chlorid of such metal, in causing the previously-added nitrosulfuric acid to react upon the said metal chlorid to form the sulfate of the metal contained in said ore, in heating to 110° to 120° centigrade to effect distillation of the aforementioned nitrochlorids, in injecting oxid-of-sulfur fumes and water-vapors to form new quantities of sulfuric acid, in causing a continuous conjoint reaction between nitrosulfuric acid, decomposable metallic chlorids, nitrochlorids, oxids-of-nitrogen fumes, oxid-of-sulfur fumes, water-vapors to form new quantities of sulfuric acid, in causing a continuous conjoint reaction between nitrosulfuric acid, decomposable metallic chlorids, nitrochlorids, oxids-of-nitrogen fumes, oxid-of-sulfur fumes, water-vapors, the metal contained in the ore and the chlorid of the said metal, in causing the cyclic formation of nitrosulfuric acid, nitrochlorids and the metal chlorid, and in causing the formation of permanent sulfate of the metal contained in the said ore.

5. The herein-described process of extracting and concentrating metals from ores consisting in treating ores with nitrosulfuric acid and decomposable metallic chlorids in closed reaction-chambers, in causing nitrosulfuric acid to react upon decomposable metallic chlorids to form nitrochlorids, in causing the said nitrochlorids to react upon the metal contained in said ore to form the chlorid of such metal, in causing the previously-added nitrosulfuric acid to react upon the said metal chlorid to form the sulfate of the metal contained in said ore, in heating to 110° to 120° centigrade to effect distillation of the aforementioned nitrochlorids, in injecting oxid-of-sulfur fumes and water-vapors to form new quantities of sulfuric acid, in causing a continuous conjoint reaction between nitrosulfuric acid, decomposable metallic chlorids, nitrochlorids, oxids-of-nitrogen fumes, oxid-of-sulfur fumes, water-vapors, the metal contained in the ore and the chlorid of said metal, in causing the cyclic formation of nitrosulfuric acid, nitrochlorids and the metal chlorid, in causing the formation of permanent sulfate of the metal contained in the said ore, in partially hydrating at 40° to 50° Baumé density and in completing the hydration with a metallic bisulfate.

6. The herein-described process of extracting and concentrating metals from ores consisting in treating ores with nitrosulfuric acid and decomposable metallic chlorids in closed reaction-chambers, in causing nitrosulfuric acid to react upon decomposable metallic chlorids to form nitrochlorids, in causing the said nitrochlorids to react upon the metal contained in said ore to form the chlorid of such metal, in causing the previously-added nitrosulfuric acid to react upon the said metal chlorid to form the sulfate of the metal contained in said ore, in heating to 110° to 120° centigrade to effect distillation of the aforementioned nitrochlorids, in injecting oxid-of-sulfur fumes and water-vapors to form new quantities of sulfuric acid, in causing a continuous conjoint reaction between nitrosulfuric acid, decomposable metallic chlorids, nitrochlorids, oxids-of-nitrogen fumes, oxid-of-sulfur fumes, water-vapors, the metal contained in the ore and the chlorid of the said metal, in causing the cyclic formation of nitrosulfuric acid, nitrochlorids and the metal chlorid, in causing the formation of permanent sulfate of the metal contained in the said ore, in partially hydrating at 40° to 50° Baumé density and in completing the hydration with sodium-bisulfate solution.

7. The herein-described process of extracting and concentrating metals from ores consisting in treating ores with nitrosulfuric acid and decomposable metallic chlorids in closed reaction-chambers, in causing nitrosulfuric acid to react upon decomposable metallic chlorids to form nitrochlorids, in causing the said nitrochlorids to react upon the metal contained in said ore to form the chlorid of such metal, in causing the previously-added nitrosulfuric acid to react upon the said metal chlorid to form the sulfate of the metal contained in said ore, in heating to 110° to 120° centigrade to effect distillation of the aforementioned nitrochlorids, in injecting oxid-of-sulfur fumes and water-vapors to form new quantities of sulfuric acid, in causing a continuous conjoint reaction between nitrosulfuric acid, decomposable metallic chlorids, nitrochlorids and the metal chlorid, in causing the formation of permanent sulfate of the metal contained in the said ore, in partially hydrating at 40° to 50° Baumé density and in completing the hydration with sodium-bisulfate solution.

8. The herein-described process of extracting and concentrating metals from ores consisting in treating ores with nitrosulfuric acid and decomposable metallic chlorids in closed reaction-chambers, in causing nitrosulfuric acid to react upon decomposable metallic chlorids to form nitrochlorids, in causing the said nitrochlorids to react upon the metal contained in said ore to form the chlorid of such metal, in causing the previously-added nitrosulfuric acid to react upon the said metal chlorid to form the sulfate of the metal contained in said ore, in heating to 110° to 120° centigrade to effect distillation of the aforementioned nitrochlorids, in injecting oxid-of-sulfur fumes and water-vapors to form new quantities of sulfuric acid, in causing a continuous conjoint reaction between nitrosulfuric acid, decomposable metallic chlorids, nitrochlorids, oxids-of-nitrogen fumes, oxid-of-sulfur fumes, water-vapors, the metal contained in the ore and the chlorid of the said metal, in causing the cyclic formation of nitrosulfuric acid, nitrochlorids and the metal chlorid, in causing the formation of permanent sulfate of the metal contained in the said ore, in partially hydrating at 40° to 50° Baumé density, in completing the hydration with a metallic bisulfate, in removing the non-metalliferous residuum from the hydrated reaction mixture.

and in saturating the remaining liquid with calcareous reagents.

8. The herein-described process of extracting and concentrating metals from ores consisting in treating ores with nitrosulfuric acid and decomposable metallic chlorids in closed reaction-chambers, in causing nitrosulfuric acid to react upon decomposable metallic chlorids to form nitrochlorids, in causing the said nitrochlorids to react upon the metal contained in said ore to form the chlorid of such metal, in causing the previously-added nitrosulfuric acid to react upon the said metal chlorid to form the sulfate of the metal contained in said ore, in heating to 110° to 120° centigrade to effect distillation of the aforementioned nitrochlorids, in injecting oxid-of-sulfur fumes and water-vapors to form new quantities of sulfuric acid, in causing a continuous conjoint reaction between nitrosulfuric acid, decomposable metallic chlorids, nitrochlorids, oxids-of-nitrogen fumes, oxid-of-sulfur fumes, water-vapors, the metal contained in the ore and the chlorid of the said metal, in causing the cyclic formation of nitrosulfuric acid, nitrochlorids and the metal chlorid, in causing the formation of permanent sulfate of the metal contained in the said ore, in partially hydrating at 40° to 50° Baumé density, in completing the hydration with a metallic bisulfate, in removing the non-metalliferous residuum from the hydrated reaction mixture and in saturating the remaining liquid with calcium carbonate and lime.

9. The herein-described process of extracting and concentrating metals from ores consisting in treating ores with nitrosulfuric acid and decomposable metallic chlorids in closed reaction-chambers, in causing nitrosulfuric acid to react upon decomposable metallic chlorids to form nitrochlorids, in causing the said nitrochlorids to react upon the metal contained in said ore to form the chlorid of such metal, in causing the previously-added nitrosulfuric acid to react upon the said metal chlorid to form the sulfate of the metal contained in said ore, in heating to 110° to 120° centigrade to effect distillation of the aforementioned nitrochlorids, in injecting oxid-of-sulfur fumes and water-vapors to form new quantities of sulfuric acid, in causing a continuous conjoint reaction between nitrosulfuric acid, decomposable metallic chlorids, nitrochlorids, oxids - of - nitrogen fumes, oxid-of-sulfur fumes, water-vapors, the metal contained in the ore and the chlorid of the said metal, in causing the cyclic formation of nitrosulfuric acid, nitrochlorids and the metal chlorid, in causing the formation of permanent sulfate of the metal contained in the said ore, in partially hydrating at 40° to 50° Baumé density, in completing the hydration with a metallic bisulfate, in removing the non-metalliferous residuum

from the hydrated reaction mixture, in saturating the remaining liquid with calcareous reagents, in separating the metalliferous calcic precipitate and in lixiviating the same with ammonia solutions.

10. The herein-described process of extracting and concentrating metals from ores consisting in treating ores with nitrosulfuric acid and decomposable metallic chlorids in closed reaction-chambers, in causing nitrosulfuric acid to react upon decomposable metallic chlorids to form nitrochlorids, in causing the said nitrochlorids to react upon the metal contained in said ore to form the chlorids of such metal, in causing the previously-added nitrosulfuric acid to react upon the said metal chlorid to form the sulfate of the metal contained in said ore, in heating to 110° to 120° centigrade to effect distillation of the aforementioned nitrochlorids, in injecting oxid-of-sulfur fumes and water-vapors to form new quantities of sulfuric acid, in causing a continuous conjoint reaction between nitrosulfuric acid, decomposable metallic chlorids, nitrochlorids, oxids-of-nitrogen fumes, oxid-of-sulfur fumes, water-vapors, the metal contained in the ore and the chlorid of the said metal, in causing the cyclic formation of nitrosulfuric acid, nitrochlorids and the metal chlorid, in causing the formation of permanent sulfate of the metal contained in the said ore, in partially hydrating at 40° to 50° Baumé density, in completing the hydration with a metallic bisulfate, in removing the non-metalliferous residuum from the hydrated reaction mixture, in saturating the remaining liquid with calcareous reagents, in separating the metalliferous calcic precipitate and in lixiviating the same with ammonia solution.

11. The herein-described process of extracting and concentrating metals from ores consisting in treating ores with nitrosulfuric acid and decomposable metallic chlorids in closed reaction-chambers, in causing nitrosulfuric acid to react upon decomposable metallic chlorids to form nitrochlorids, in causing the said nitrochlorids to react upon the metal contained in said ore to form the chlorid of such metal, in causing the previously-added nitrosulfuric acid to react upon the said metal chlorid to form the sulfate of the metal contained in said ore, in heating to 110° to 120° centigrade to effect distillation of the aforementioned nitrochlorids, in injecting oxid-of-sulfur fumes and water-vapors to form new quantities of sulfuric acid, in causing a continuous conjoint reaction between nitrosulfuric acid, decomposable metallic chlorids, nitrochlorids, oxids-of-nitrogen fumes, oxid-of-sulfur fumes, water-vapors, the metal contained in the ore and the chlorid of the said metal, in causing the cyclic formation of nitrosulfuric acid, nitrochlorids and the metal chlorid, in causing the formation of permanent sulfate of the metal contained in the said ore, in partially hydrating at 40° to 50° Baumé density, in completing the hydration with a metallic bisulfate, in removing the non-metalliferous residuum from the hydrated reaction mixture, in saturating the remaining liquid with calcareous reagents, in separating the metalliferous calcic precipitate and in lixiviating the same with ammonia solution.

tion of permanent sulfate of the metal contained in the said ore, in partially hydrating at 40° to 50° Baumé density, in completing the hydration with a metallic bisulfate, in removing the non-metalliferous residuum from the hydrated reaction mixture, in saturating the remaining liquid with calcareous reagents, in separating the metalliferous calcic precipitate, in lixiviating the same with ammonia solutions, in removing the calcareous sediment and in distilling the lixiviation fluid until freed from hydrogen nitrid.

12. The herein-described process of extracting and concentrating metals from ores consisting in treating ores with nitrosulfuric acid and decomposable metallic chlorids in closed reaction-chambers, in causing nitrosulfuric acid to react upon decomposable metallic chlorids to form nitrochlorids, in causing the said nitrochlorids to react upon the metal contained in said ore to form the chlorid of such metal, in causing the previously-added nitrosulfuric acid to react upon the said metal chlorid to form the sulfate of the metal contained in said ore, in heating to 110° to 120° centigrade to effect distillation of the aforementioned nitrochlorids, in injecting oxid-of-sulfur fumes and water-vapors to form new quantities of sulfuric acid, in causing a continuous conjoint reaction between nitrosulfuric acid, decomposable metallic chlorids, nitrochlorids, oxids-of-nitrogen fumes, oxid-of-sulfur fumes, water-vapors, the metal contained in the ore and the chlorid of the said metal, in causing the cyclic formation of nitrosulfuric acid, nitrochlorids and the metal chlorid, in causing the formation of permanent sulfate of the metal contained in the said ore, in partially hydrating at 40° to 50° Baumé density, in completing the hydration with a metallic bisulfate, in removing the non-metalliferous residuum from the hydrated reaction mixture, in saturating the remaining liquid with calcareous reagents, in separating the metalliferous calcic precipitate, in lixiviating the same with ammonia solutions, in removing the calcareous sediment, in distilling the lixiviation fluid until freed from the ammonia, and in separating the hydrated metallic oxides precipitated thereby.

13. The herein-described process of extracting and concentrating metals from ores consisting in treating ores with nitrosulfuric acid and decomposable metallic chlorids in closed reaction-chambers, in causing nitrosulfuric acid to react upon decomposable metallic chlorids to form nitrochlorids, in causing the said nitrochlorids to react upon the metal contained in said ore to form the chlorid of such metal, in causing the previously-added nitrosulfuric acid to react upon the said metal chlorid to form the sulfate of the metal contained in said ore, in heating to 110° to 120° centigrade to effect distillation

of the aforementioned nitrochlorids, in injecting oxid-of-sulfur fumes and water-vapors to form new quantities of sulfuric acid, in causing a continuous conjoint reaction between nitrosulfuric acid, decomposable metallic chlorids, nitrochlorids, oxids-of-nitrogen fumes, oxid-of-sulfur fumes, water-vapors, the metal contained in the ore and the chlorid of the said metal, in causing the cyclic formation of nitrosulfuric acid, nitrochlorids and the metal chlorid, in causing the formation of permanent sulfate of the metal contained in the said ore, in recovering the aforesaid nitrochlorids by distillation and in using the same in subsequent decompositions of ores in place of new charges thereof.

14. The herein-described process of extracting and concentrating metals from ores consisting in treating ores with nitrosulfuric acid and decomposable metallic chlorids in closed reaction-chambers, in causing nitrosulfuric acid to react upon decomposable metallic chlorids to form nitrochlorids, in causing the said nitrochlorids to react upon the metal contained in said ore to form the chlorid of such metal, in causing the previously-added nitrosulfuric acid to react upon the said metal chlorid to form the sulfate of the metal contained in said ore, in heating to 110° to 120° centigrade to effect distillation of the aforementioned nitrochlorids, in injecting oxid-of-sulfur fumes and water-vapors to form new quantities of sulfuric acid, in causing a continuous conjoint reaction between nitrosulfuric acid, decomposable metallic chlorids, nitrochlorids, oxids-of-nitrogen fumes, oxid-of-sulfur fumes, water-vapors, the metal contained in the ore and the chlorid of the said metal, in causing the cyclic formation of nitrosulfuric acid, nitrochlorids and the metal chlorid, in causing the formation of permanent sulfate of the metal contained in the said ore, in partially hydrating at 40° to 50° Baumé density, in completing the hydration with a metallic bisulfate, in removing the non-metalliferous residuum from the hydrated reaction mixture, in saturating the remaining liquid with calcareous reagents, in separating the metalliferous calcic precipitate, in lixiviating the same with ammonia solutions, in removing the calcareous sediment, in recovering the residual ammonia from the said calcareous sediment and in using the recovered ammonia in subsequent lixiviations in place of new charges thereof.

15. The herein-described process of extracting and concentrating metals from ores consisting in treating ores with nitrosulfuric acid and decomposable metallic chlorids in closed reaction-chambers, in causing nitrosulfuric acid to react upon decomposable metallic chlorids to form nitrochlorids, in causing the said nitrochlorids to react upon the metal contained in said ore to form the

- chlorid of such metal, in causing the previously-added nitrosulfuric acid to react upon the said metal chlorid to form the sulfate of the metal contained in said ore, in heating to 5 110° to 120° centigrade to effect distillation of the aforementioned nitrochlorids, in injecting oxid-of-sulfur fumes and water-vapors to form new quantities of sulfuric acid, in causing a continuous conjoint reaction between 10 nitrosulfuric acid, decomposable metallic chlorids, nitrochlorids oxids-of-nitrogen fumes, oxid-of-sulfur fumes, water-vapors, the metal contained in the ore and the chlorid of the said metal, in causing the cyclic formation of nitrosulfuric acid, nitrochlorids and the metal chlorid, in causing the formation of permanent sulfate of the metal contained in the said ore, in partially hydrating at 40° to 50° Baumé density, in completing 15 the hydration with a metallic bisulfate, in removing the non-metalliferous residuum from the hydrated reaction mixture, in saturating the remaining liquid with calcareous reagents, in separating the metalliferous calcic precipitate, in lixiviating the same with ammonia solutions, in removing the calcareous sediment, in distilling the lixiviation fluid until freed from ammonia, in recovering the said distilled ammonia and in using the same in 20 subsequent lixiviations in place of new charges thereof.
16. The herein-described process of extracting and concentrating nickel from silicious nickel ore, consisting in treating said ore with nitrosulfuric acid and sodium chlorid in closed reaction-chambers, in causing nitrosulfuric acid to react upon sodium 25
- chlorid to form nitrochlorids, in causing the said nitrochlorids to react upon the nickel contained in said ore to form chlorid of nickel, 40 in causing the previously-added nitrosulfuric acid to react upon the said nickel chlorid to form sulfate of the nickel contained in said ore, in heating to 110° to 120° centigrade to effect distillation of the aforementioned nitrochlorids, in injecting oxid-of-sulfur fumes and water-vapors to form new quantities of sulfuric acid, in causing a continuous conjoint reaction between nitrosulfuric acid, sodium chlorid, nitrochlorids, oxids - of - nitrogen fumes, oxid-of-sulfur fumes, water-vapors, the nickel of said ore and chlorid of nickel, in causing the cyclic formation of nitrosulfuric acid, nitrochlorids and nickel chlorid, in causing formation of permanent sulfate of the nickel contained in said ore, in partially hydrating at 40° to 50° Baumé density, in completing the hydration with sodium bisulfate solution, in removing the non-metalliferous residuum of the silicious ore from the hydrated reaction mixture, in saturating the remaining liquid with calcium carbonate and lime, in separating the metalliferous calcic precipitate, in lixiviating the same with ammonia solutions, in removing the calcareous sediment, in distilling the lixiviation solution until freed from ammonia and in separating the hydrated nickel oxid 55 precipitated thereby.
- In testimony whereof I have hereunto set my hand in presence of two witnesses.
- DENIS LANCE.
- Witnesses:
- ADOLPHE STURM,  
HANSON C. COXE.